

## UNITED STATES PATENT OFFICE

2,143,760

METHOD AND COMPOSITION FOR  
CADMIUM PLATING

Leroy Camel, Maple Heights, Ohio, assignor to  
The Plating and Galvanizing Company, Cleve-  
land, Ohio, a corporation of Ohio

No Drawing. Application December 11, 1936,  
Serial No. 115,349

## 12 Claims.

(Cl. 204—1)

This invention, as indicated, relates to a method and composition for cadmium plating, especially in relation to ferrous articles. More particularly, it comprises a composition having a combination of elements adapted to bring about a bright plating of cadmium or cadmium associated with other metals or alloys and providing a method adaptable for quantity production with a product of uniform quality and dependable finish.

Various types of cadmium plating compositions and processes are known, but many of these are not adapted for commercial use, either because of cost or intricacy of handling, or by reason of difficulty in maintaining uniformity of product.

The present invention utilizes a cyanide bath as the electrolyte and includes with the same, small quantities of compounds to improve the conductivity of the bath and to bring about a bright coating upon the articles being plated. It has been found that the cyanide bath in general results in the best quality of color for the product, but in many instances the time factor of the operation has been poor or the control of the operation has been difficult. With the composition herein described, it has been found that a uniformly high rate of production can be maintained and a cadmium coating of high luster maintained on the product, with no unfavorable factors to be taken into account as to the maintenance of the bath or excessive cost or complication in carrying out the process.

The process, while adapted to be carried out in certain proportionate relations between the elements entering into the same, is by no means restricted to certain critical proportions, but has a reasonable range of limits as to quantities, as well as to substitution of equivalent elements.

The compounds used for the electrolyte may comprise the following substances in proportions varying between the limits indicated:

## Sodium cyanide

ounces per gallon of water 10 to 15

45 Cadmium oxide or hydrate do 4 to 7

Sodium sulphate do 3 to 6

Sodium sulphite do 25 to 1

Silver or cobalt salts do .133 to .2

Tung oil do 25 to 1

50 Water gallon 1

As a thoroughly tested cadmium plating bath

for producing high luster cadmium coatings, the following formula is set forth:

|                 |                            |      |    |
|-----------------|----------------------------|------|----|
| Sodium cyanide  | ounces per gallon of water | 13   |    |
| Cadmium oxide   | do                         | 5    | 5  |
| Sodium sulphate | do                         | 5.2  |    |
| Sodium sulphite | do                         | .25  |    |
| Silver nitrate  | do                         | .133 |    |
| Tung oil        | do                         | .25  |    |
| Water           | gallon                     | 1    | 10 |

While tung oil is preferred as an addition agent, other oils such as cod liver oil or the like may be utilized, the oil preferably being an oil having a high degree of tenacity in the form of a thin film.

Likewise, while a small amount of silver is found most effective in securing a bath having a high production efficiency, it has been found that cobalt may also be used satisfactorily. The quantities set forth, as stated, are not critical.

If desired, however, a mixture in dry form of all of the ingredients except the tung oil may be prepared, such ingredients being added to the water which may be very moderately heated to assist in the full dissolution of the powdered material and thereafter the tung oil added to such solution.

The bath, when fully prepared, will be found to permit the use of a current of up to 45 amperes in the plating circuit or as low as 10 amperes per square foot of surface at preferably from 3 to 5 volts. The anode utilized preferably comprises pure cadmium, although anodes partially formed of cadmium may be utilized under special conditions. The remaining portion of the anode in such instances may include silver or non-active material. At a temperature of between 60° and 90° Fahrenheit, the plating bath above set forth will coat ferrous articles with a satisfactory coating in approximately from four to six minutes, and such coating will be closely adherent to the surface treated, of fine grain, and of smooth bright texture.

The articles when plated as above outlined may be utilized for many purposes as a final coating without buffing or finishing treatment of any character, or the coating so provided may form a base coating for a finishing coat of other metal such as nickel or the like.

Other modes of applying the principle of my invention may be employed instead of those explained, change being made as regards the means and steps herein disclosed, provided the means stated by any of the following claims or the equivalent of such stated means be employed.

I therefore particularly point out and distinctly claim as my invention:

1. The process of producing bright smooth 10 coatings of cadmium on ferrous articles in an alkali cyanide solution, which comprises the steps of adding to the alkali electrolytic bath a substance containing sodium sulphite and tung oil, and suspending in said bath at the respective terminals of the plating circuit a cadmium anode and the article to be plated.

2. A composition of matter adapted for use in forming an electrolyte for the electrodeposition of cadmium, consisting of substantially 13 ounces of sodium cyanide, 5 ounces of cadmium oxide, 5.2 ounces of sodium sulphate, .25 ounce of sodium sulphite, .133 ounce of silver nitrate, and .25 ounce of tung oil to each gallon of water used for said electrolyte.

3. The process of electrolytically coating a ferrous article with cadmium in an alkali cyanide solution which consists in passing an electric current through said article as a cathode in the presence of a cadmium anode and an electrolyte containing sodium sulphite and a silver salt in less amount than any other substance in said electrolyte, said electrolyte containing an addition agent in the form of an oil of high film tenacity from a group consisting of tung oil and cod liver oil.

4. The process of electrolytically coating a ferrous article with cadmium in an alkali cyanide solution which consists in passing an electric current through said article as a cathode in the presence of a cadmium anode and an alkali cyanide electrolyte containing sodium sulphite and an addition agent from the group consisting of tung oil and cod liver oil.

5. In the art of cadmium plating, the process 45 which comprises electroplating cadmium from an alkali cyanide bath containing sodium sulphite in the presence of an addition agent selected from the group consisting of tung oil and cod liver oil.

6. In the art of cadmium plating, the process which comprises electroplating cadmium from an alkali cyanide bath in the presence of sodium sulphite, a metallic salt from the group consisting of silver and cobalt, such salt being in amount less than any other substance in said electrolytic

bath, and an addition agent from the group consisting of tung oil and cod liver oil.

7. The process of producing bright smooth 5 coatings of cadmium on ferrous articles in an alkali cyanide solution which comprises the steps of adding to the electrolytic bath sodium sulphite and an oil of high film tenacity from a group consisting of tung oil and cod liver oil and suspending in said bath at the respective terminals of the plating circuit a cadmium anode and the 10 article to be plated.

8. A sodium cadmium cyanide bath for electroplating with cadmium or cadmium associated with other metals comprising in combination sodium sulphite to the amount of approximately 15 .25 ounce per gallon of water, an oil selected from the group consisting of tung oil and cod liver oil, and a salt of silver adding electrical conductivity to said bath.

9. In a sodium cadmium cyanide bath for electroplating with cadmium or cadmium associated with other metals, the combination of tung oil to the amount of approximately .25 ounce per gallon of water, sodium sulphite and a salt of silver adding electrical conductivity to said bath.

10. In a sodium cadmium cyanide bath for electroplating with cadmium or cadmium associated with other metals, the combination of sodium sulphite to the amount of approximately .25 ounce per gallon of water and tung oil to the amount of approximately .25 ounce per gallon of water.

11. In a sodium cadmium cyanide bath for electroplating with cadmium or cadmium associated with other metals, the combination of sodium sulphite to the amount of approximately .25 ounce per gallon of water, tung oil to the amount of approximately .25 ounce per gallon of water, and silver nitrate to the amount of .133 ounce per gallon of water.

12. A composition of matter adapted for use 40 in forming an electrolyte for the electrodeposition of cadmium consisting, for each gallon of water to be used, of the proportion of 10 to 15 ounces of sodium cyanide, 4 to 7 ounces of cadmium compound selected from a group consisting of cadmium oxide and cadmium hydrate, 3 to 6 ounces of sodium sulphate, .25 to 1 ounce of sodium sulphite, .133 to .2 ounce of a salt of a metal from the group consisting of silver and cobalt, and .25 to 1 ounce of an oil of high film tenacity taken from the group consisting of tung oil and cod liver oil.

LEROY CAMEL.